

## UNITED STATES PATENT OFFICE

1,930,910

## TANNING SOLUTION

Otto Röhm, Darmstadt, Germany

No Drawing. Application May 15, 1928, Serial  
No. 278,045, and in Germany June 20, 1927

9 Claims. (Cl. 149—5)

I have filed an application for patent in Germany on June 20, 1927.

My invention relates to mineral tanning and consists in the discovery that salts of iron, or 5 chromium, or aluminum, or several salts of these, on the one hand, and phosphoric acid or acids of arsenic, or salts or esters of said acids can be advantageously employed for mineral tannage.

To name some of the salts, by way of example, 10 I would mention in the first place, the chlorides and sulfates, whereas of the salts of phosphoric acid I would mention the sodium phosphate and of the esters, for instance, the glycerine phosphoric acid, eventually in combination with alkali 15 or alkaline earth metals.

## Example 1

20 kilograms of iron sulfate chloride to which 1 kilogramme of phosphoric acid has been 20 added are dissolved in 25 liters of water. To this are added, while the solution is continually stirred, 170 liters of water wherein are contained 4.2 kilograms of neutral sodium carbonate. With this tanning liquor 100 kilograms of pelts 25 are tanned by being moved around for 6 to 8 hours in the tanning vessel.

## Example 2

5 kilograms of alum, to which are added 3 30 kilograms of common salt and 0.5 kilograms of glycerine phosphoric acid are dissolved in 100 liters of water, and in this solution 100 kilograms of pelts are tanned by being moved around for 6 to 8 hours in the tanning vessel.

## Example 3

20 kilograms of iron sulfate chloride are dissolved in 25 liters of water to which have been 40 added 1.75 kilogramme of glycerine phosphoric acid. After the solution is completed 170 kilograms of a 1.8% soda solution are added during stirring. In this solution 100 kilograms of pelts are tanned by being moved around in the tanning vessel for 6-8 hours.

## Example 4

10 kilograms of crystallized chromium chloride are dissolved in 100 liters of water to which 3 kilograms of common salt have been added. 50 To this solution I add 0.3 kilogramme of 100% anhydrous glycerophosphate of sodium and gradually 2 kilograms of calcinated soda during stirring. In this liquor 100 kilograms of pelts are tanned by being moved in the tanning 55 vessel for 4-6 hours.

The phosphoric acid, or the acids of arsenic, or the corresponding salts or esters can be added either during the tanning operation, or can be used already in the pickle, or they can be used in the stuffing.

There is already known a chromium two-baths tanning process, in which arsenic salts are used, which process I expressly disclaim. Also tanning processes have been described in which iron and chromium compounds as well as pyro-phosphates 65 are used, in which processes it is necessary to also use boron, wherein said processes differ from my process.

What I claim is:

1. A tanning solution, comprising iron salts 70 containing a trivalent cation, and esters of phosphoric acid.

2. A tanning solution, comprising chromium salts containing a trivalent cation, and esters of phosphoric acid. 75

3. A tanning solution, comprising aluminum salts containing a trivalent cation, and esters of phosphoric acid.

4. A tanning solution, comprising iron salts 80 containing a trivalent cation and salts of the esters of phosphoric acid.

5. A tanning solution, comprising chromium salts containing a trivalent cation, and salts of the esters of phosphoric acid.

6. A tanning solution, comprising aluminum 85 salts containing a trivalent cation, and salts of the esters of phosphoric acid.

7. A tanning solution, comprising iron sulfate chloride and phosphoric acid.

8. A tanning solution, comprising aluminum 90 salts and glycerine phosphoric acid.

9. A tanning solution, comprising a chromium salt and sodium glycerine phosphate.

OTTO RÖHM.

95

100

105

110